

ing one head or another to the generator, a plurality of control elements at the heads for controlling the radio frequency switches, means including a shaft for varying the voltage output of the radio frequency generator, a motor for moving said shaft, a plurality of discs frictionally secured to the shaft, a toothed stop element secured to said shaft, a pawl for engaging and locking said stop element, cam rollers engaging said discs, said discs being recessed to receive the rollers to mark a desired stopping point depending on the adjustment of the disc relative to the shaft and corresponding to the desired radio frequency voltage for the corresponding head, and detent means to hold out and make inoperative the rollers, each of the aforesaid control elements serving to close a radio frequency switch, and to start the motor in order to rotate the aforesaid shaft in forward direction, and to release and make operative a cam roller which on entering the cam depression changes the position of a switch and thereby stops the motor and operates the locking pawl.

14. Pill heating apparatus for use with a plurality of molding presses using a plurality of different size pills, said apparatus comprising a heating head for each press, a radio frequency generator, radio frequency switches for connecting one head or another to the generator, a plurality of control elements at the heads for controlling relay circuits, means including a shaft for varying the voltage output of the radio frequency generator, a motor for moving said shaft, a plurality of discs frictionally secured to the shaft, a toothed stop element secured to said shaft, a pawl for engaging and locking said stop element, cam rollers engaging said discs, said discs being recessed to receive the rollers to mark a desired stopping point depending on the adjustment of the disc relative to the shaft and corresponding to the desired radio frequency voltage for the corresponding head, detent means to hold out and make inoperative the rollers, and a timing clock for timing the heating of the pills, each of the aforesaid relay circuits serving to close a radio frequency switch, and to start the motor in order to rotate the shaft in forward direction, and to start the timing clock, and to release and make operative a cam roller which on entering the cam depression changes the position of a switch and thereby stops the motor and operates the locking pawl, running out of said timing clock serving to oppositely change said relay circuit and to thereby release the pawl, to reverse the motor, to restore the roller to the detent means, and to open the radio frequency switch.

15. Pill heating apparatus for use with a plurality of molding presses using a plurality of different size pills, said apparatus comprising a heating head for each press, a radio frequency generator, radio frequency switches for connecting one head or another to the generator, a plurality of control elements at the heads for controlling the radio frequency switches, a low frequency power supply for the radio frequency generator including a variable transformer or variac for varying the voltage output of the radio frequency generator, a motor for driving the variac shaft through reduction gearing, a plurality of discs frictionally secured to the variac shaft, a toothed stop element secured to said shaft, a pawl for engaging and locking said stop element, cam rollers engaging said discs, said discs being recessed to receive the rollers to mark a desired stopping point depending on the ad-

justment of the disc relative to the shaft and corresponding to the desired radio frequency voltage for the corresponding head, and detent means to hold out and make inoperative the rollers, each of the aforesaid control elements serving to close a radio frequency switch, and to start the motor in order to rotate the variac in forward direction, and to release and make operative a cam roller which on entering the cam depression changes the position of a switch and thereby stops the motor and operates the locking pawl.

16. Pill heating apparatus for use with a plurality of molding presses using a plurality of different size pills, said apparatus comprising a heating head for each press, a radio frequency generator, radio frequency switches for connecting one head or another to the generator, a plurality of control elements at the heads for controlling relay circuits, a low frequency power supply for the radio frequency generator including a variable transformer or variac for varying the voltage output of the radio frequency generator, a motor for driving the variac shaft through reduction gearing, a plurality of discs frictionally secured to the variac shaft, a toothed stop element secured to said shaft, a pawl for engaging and locking said stop element, cam rollers engaging said discs, said discs being recessed to receive the rollers to mark a desired stopping point depending on the adjustment of the disc relative to the shaft and corresponding to the desired radio frequency voltage for the corresponding head, detent means to hold out and make inoperative the rollers, and a timing clock for timing the heating of the pills, each of the aforesaid relay circuits serving to close a radio frequency switch, and to start the motor in order to rotate the variac in forward direction, and to start the timing clock, and to release a cam roller which on entering the cam depression changes the position of a switch and thereby stops the motor and operates the locking pawl, running out of said timing clock serving to oppositely change said relay circuit and to thereby release the pawl, reverse the motor, restore the roller to the detent means, and open the radio frequency switch.

17. A remotely controlled mechanism for moving a variac or like control device from zero to any of several different desired positions, said mechanism including a motor to drive the variac shaft, a switch to control the operation of the motor, a toothed wheel positively secured to said shaft, a pawl for engaging the teeth of said wheel to stop and lock the shaft, a plurality of cams frictionally rotatable on said shaft, each of said cams having a stop depression and being independently rotatively adjustable on the shaft to a desired position, a plurality of cam rollers for engaging said cams, a detent for normally holding said cam rollers in inoperative position, means for selecting and releasing one of said cam rollers from said detent to operative position, said cam roller on entering the stop depression of its associated cam serving to change the position of said motor switch and thereby serving to deenergize the motor and to actuate said locking pawl, and additional means to facilitate adjusting the desired stop positions of the cams, said means including a position locking means for so positively holding the selected cam roller in its stop depression that it is not forced out by attempted rotation of the cam, means for making said locking pawl inoperative, and a handle on said variac shaft for forcibly rotating the shaft and with it all but one of the cams, the excepted cam being

locked against rotation by the aforesaid cam roller and locking means.

18. Pill heating apparatus for use with a plurality of molding presses using a plurality of different size pills, said apparatus comprising a heating head for each press, a single radio frequency generator, switches for connecting one head or another to the generator, a plurality of control elements, voltage control means for varying the voltage output of the generator, a motor 10 for driving said voltage control means, a plurality of different independently selectable stop means for stopping movement of said voltage control means at a desired point, means to independently adjust the stop position of each of said stop means, a timing clock for timing the heating of the pills, each of the aforesaid control elements serving to close one of the switches and to start the motor in order to move the voltage control means in forward direction and to start the timing clock and to make one of the stop means operative, said stop means stopping the motor at the desired voltage output, and running out of said timing clock serving to reverse the motor and open the switch.

5

20

25

GORDON B. SAYRE.

## REFERENCES CITED

The following references are of record in the file of this patent:

## UNITED STATES PATENTS

| Number    | Name              | Date          |
|-----------|-------------------|---------------|
| 1,513,681 | Ward              | Oct. 28, 1924 |
| 2,036,516 | Golanduoni        | Apr. 7, 1936  |
| 2,085,442 | Newell            | June 29, 1937 |
| 2,094,777 | Ellinger          | Oct. 5, 1937  |
| 2,102,070 | Harris            | Dec. 14, 1937 |
| 2,153,865 | Gersch            | Apr. 11, 1939 |
| 2,234,911 | Davis             | Mar. 11, 1941 |
| 2,251,277 | Hart, Jr., et al. | Aug. 5, 1941  |
| 2,275,284 | Carlson           | Mar. 3, 1942  |
| 2,280,766 | Bronaugh          | Apr. 21, 1942 |
| 2,293,851 | Rogers            | Aug. 25, 1942 |
| 2,334,724 | Paessler          | Nov. 23, 1943 |
| 2,367,763 | Elliott           | Jan. 23, 1945 |
| 2,391,470 | May               | Dec. 25, 1945 |
| 2,401,277 | Stratton          | May 28, 1946  |
| 2,401,991 | Walton et al.     | June 11, 1946 |
| 2,403,800 | Hoyler            | July 9, 1946  |
| 2,415,799 | Riefel et al.     | Feb. 11, 1947 |
| 2,419,307 | Zottu             | Apr. 22, 1947 |
| 2,490,619 | Clark             | Dec. 6, 1949  |
| 2,506,814 | Sayre             | May 9, 1950   |

## UNITED STATES PATENT OFFICE

2,583,394

## EXTREME PRESSURE GREASES

John E. Schott, New York, and Eldon L. Armstrong, Garden City, N. Y., assignors to Socony-Vacuum Oil Company, Incorporated, a corporation of New York

No Drawing. Application September 20, 1950,  
Serial No. 185,913

9 Claims. (Cl. 252—36)

1

This is a continuation-in-part of our co-pending application, Serial Number 79,518, filed March 3, 1949 for High Temperature Extreme Pressure Greases, now abandoned.

This invention relates to an improved method for preparing improved lubricating grease compositions useful for high pressure service. It is directed to improved methods of preparing greases based upon soaps of the alkaline earth metals, and particularly directed to an improved method for preparing a lime-base grease containing a lead soap, and metal salts of low molecular weight mono-basic fatty acids.

The greases prepared by the method of this invention are well adapted for extreme pressure service where high unit loads are encountered, for example in the lubrication of roller bearings in steel mills. A lime base grease made according to this procedure is also adapted for use at temperatures going up to about 300—325° F. which is substantially higher than those at which ordinary calcium base greases may be employed.

An object of this invention is the provision of an economical and efficient method for making improved greases which utilize for bases the soaps of alkaline earth metals, e. g., calcium, barium, magnesium and strontium, and which contain extreme pressure ingredients and improving amounts of metal salts of low molecular weight monobasic fatty acids. An object of this invention is the provision of an efficient, rapid and economical process for making calcium-lead soap greases. Another object is the provision of an improved lubricant for extreme pressure service containing calcium and lead soaps. These and other objects of this invention will become apparent from the following discussion.

Heretofore, in preparing lead greases containing the soaps of lead and another metal, it has been customary to first prepare a grease containing the other metal and then to add thereto a separately prepared lead soap or soaps followed by extended heating of the mixture to accomplish proper distribution of the lead soaps therein. For example, in the case of an alkali base soap, a sodium base grease is first prepared by methods well known to the art and a lead soap, for example lead oleate prepared by reacting litharge with oleic acid, is added and gradually worked into the sodium base grease. It has now been found that a very good lime base grease may be prepared by mixing together at atmospheric temperature the saponifiable material with litharge and lime and a mono-basic fatty acid such as acetic acid followed by heating under pressure to effect simultaneous saponification of all the materials. This is followed by a dehydration step. This method has been found not only to provide a superior more stable grease but results in substantial manufacturing economies and ad-

vantages not found in prior art methods. Since this method permits the addition of acetic acid at room temperature to the kettle batch prior to saponification, the partial loss thereof by vaporization which has been encountered in prior grease manufacturing methods is avoided. Also, the separate preparation of metal acetates followed by inefficient mixing thereof into the formed grease is avoided.

It has been found that this same method may be followed in the preparation of similarly formulated greases utilizing as base soaps the soaps of the other alkaline earth metals, viz. barium, magnesium and strontium, as well as calcium, or mixtures of the same.

As an example of the method of this invention the preparation of a typical batch of preferred composition will be described. A pressure kettle of the type conventionally employed for such purposes is charged as follows:

## EXAMPLE I

|                                                                              | Pounds |
|------------------------------------------------------------------------------|--------|
| Tallow                                                                       | 625    |
| Glycerine                                                                    | 110    |
| Candelilla wax                                                               | 90     |
| Oleic acid                                                                   | 330    |
| Lime flour $\text{Ca}(\text{OH})_2$                                          | 270    |
| Acetic acid                                                                  | 180    |
| Water                                                                        | 150    |
| Paraffin oil (300" at 100° F. Saybolt)                                       | 1,300  |
| Litharge slurry dispersed in 35 gallons of 300" paraffin oil wt. of litharge | 173    |

After the pressure kettle has been charged with all of the above materials at about atmospheric temperature, the mixture is heated slowly while mixing to about 300° F. at which temperature substantially complete saponification is accomplished. It is desirable to maintain the kettle under pressure during the saponification step. A pressure of 60 pounds gauge has been found to be satisfactory. The saponification is completed in about two hours after which the contents of the pressure kettle are blown over into an open kettle and about 194 gallons of 100" at 100° F. paraffin oil are added while paddling the mixture. Then while continuing the mixing by paddles, steam is turned into the kettle jacket and the mixture is heated gradually to about 250° F. at atmospheric pressure after which it is rapidly heated to about 300° F. By this procedure dehydration is effected to a degree sufficient to insure high temperature stability of the final grease. The mixture is maintained at 300—310° F. for one and one half hours and then it is cut back slowly with about 44 gallons of 300" at 100° F. S. U. V. paraffin oil followed by about 100 gallons of 200" at 210° F. Mid-Continent oil. The latter oil is added only as fast as it will flow from the small bung opening of a standard 50 gallon steel

barrel. Then, the mixture is further cut back by adding more rapidly an additional 250 gallons of the 200" at 210° F. S. U. V. Mid-Continent oil. During the cut-back operation, steam is maintained in the jacket. The steam is finally turned off with the mixture at about 290-300° F. and 500 pounds of sulfurized fatty oil are added while mixing. (The sulfurized fatty oil is prepared by heating a fatty oil such as lard oil or sperm oil with about 10 percent of its weight of sulfur for about 3 hours at a temperature above about 200° F.) Finally up to 100 gallons of 300" at 100° F. S. U. V. paraffin oil is added to adjust the batch to the desired penetration grade. Cold water is then admitted to the jacket and the grease is cooled to about 180° F. for filling into packages. In preparing this grease the total material compounded together breaks down as follows:

|                              | Percent weight |
|------------------------------|----------------|
| Tallow                       | 6.7            |
| Candelilla wax               | 1.0            |
| Ca(OH) <sub>2</sub>          | 2.7            |
| PbO                          | 1.8            |
| Acetic acid                  | 1.9            |
| Glycerine                    | 2.0            |
| Oleic acid                   | 3.6            |
| Water (less than)            | 0.5            |
| Mineral oil                  | 74.8           |
| Sulfurized fatty oil (10% S) | 5.0            |
|                              | 30             |
|                              | 100.0          |

The total time consumed in preparation of this grease is about 10-12 hours. The resulting grease is of excellent consistency and is stable under service at very high unit load pressures. Moreover, due to the presence of calcium acetate, the grease has remarkable high temperature characteristics as indicated by an A. S. T. M. drop point higher than about 400° F. For purposes of comparison the grease prepared in the manner described hereinabove will be referred to herein-after as Process A grease.

The advantages of the above process over those of the prior art and the improvement in the properties of the resulting grease as compared with prior art alkali base-lead soap greases are very marked. In order to reduce the number of variables and to emphasize the importance of the procedure of effecting simultaneous saponification of fats or fatty acids with lime and litharge together, the process of this invention may be best contrasted with a process wherein a lime base-lead soap grease is prepared following the manufacturing procedure employed by the prior art in preparing lead greases containing a lead soap in addition to another metal. Using the manufacturing process procedure of the prior art, a pressure kettle was charged as follows:

#### EXAMPLE II

|                                               |        |     |
|-----------------------------------------------|--------|-----|
| Tallow                                        | pounds | 625 |
| Candelilla wax                                | do     | 180 |
| Lime flour (Ca(OH) <sub>2</sub> )             | do     | 240 |
| Water                                         | do     | 165 |
| Paraffin oil 300" at 100° F. S. U. V. gallons | 176    | 65  |

Saponification was effected at about 300° F. and 60 pounds per square inch in about two hours. The kettle contents were then blown over to an open kettle and 110 gallons of 300" at 100° F. S. U. V. paraffin oil was added while mixing. The mixture was cooled to about 120° F. and 110 pounds of glycerine and 180 pounds of acetic acid were added. The kettle contents were mixed by paddling for about 45 minutes after which the mixture was heated to about 300° F.

to effect dehydration. The dehydration step required about 5 hours. About 90 gallons of 100" at 100° F. S. U. V. paraffin oil and 75 gallons of 200" at 210° F. S. U. V. Mid-Continent oil were added to the mixture. Then about 70 pounds of lime flour, Ca(OH)<sub>2</sub> mixed in 35 gallons of 100" at 100° F. S. U. V. paraffin oil were added. The kettle contents were mixed for a half hour after which a lead oleate concentrate was added. The lead oleate concentrate consisted of about 60 percent of lead oleate and 40 percent of 100" at 100° F. S. U. V. paraffin oil. The lead oleate concentrate was prepared separately by reacting litharge with oleic acid in the presence of mineral oil. About 330 gallons of 200" at 210 S. U. V. Mid-Continent oil and 90 gallons of 100" at 100° F. S. U. V. paraffin oil were then added and the mixture was heated to about 300-320° F. and mixed for about 4 hours to effect distribution of the lead oleate in the mixture. Then 500 pounds of sulfurized fatty oil were added to the mixture followed by mixing for another half hour. The grease was then cooled for packaging. The required time consumed in preparing this grease was about 22 hours. The grease from this latter process will be referred to hereinafter as Process B grease.

Applicants are not aware of a prior art lead containing grease in which metal acetates have been employed. Metal acetates have been employed in certain other types of greases and in such instances it has been the practice to follow one of two procedures. In the first method the metal acetates have been separately formed and then added by mixing into the formed grease. Poor uniformity of mixing often results from this procedure. The second procedure has been to add acetic acid to the batch after the saponification step and prior to the dehydration step. The batch is hot at this stage of the process and a loss by vaporization of part of the added acetic acid occurs. This results in inaccurate control of the amount of metal acetates finally formed. It will be apparent that applicants' method avoids the disadvantages of the prior art methods.

The greases prepared by the above described methods were tested for storage stability, shear stability and Timken O. K. load ratings. The storage stability of the greases was determined by running worked and unworked penetrations on samples of the grease before and after storage, employing the standard A. S. T. M. procedure outlined in A. S. T. M. test D-217-44T and using a 150 gram cone. The shear test was conducted by subjecting a grease sample to a continuous shear condition for a period of three and one half hours after which A. S. T. M. penetrations were run on the grease. The shear testing system consists of a grease reservoir of greater than 10 pounds of grease capacity. The reservoir is piped to a piston pump which draws the grease from the reservoir. The high pressure side of the pump is piped to a relief valve set for maintaining about 2000 pounds per square inch gauge pressure. The grease is forced through the relief valve and then passes through about 32 feet of one inch pipe back to the reservoir where it is again picked up by the pump for recirculation. After three and one half hours circulation, the grease is removed from the shear tester and evaluated for worked and unworked penetrations. The values so obtained are compared with those of the original grease before the shear test. The spread in values represents an approximate measure of what might be ex-

pected when the greases are subjected in use to high shearing pressures. The load test is one originally developed by the Timken Roller Bearing Company of Canton, Ohio, for testing the load carrying capacity of lubricants. This test is discussed in Klemgard's Lubricating Greases, 1937 edition, page 828 and the apparatus is described by E. Wooler, in Society of Automotive Engineers' Journal, volume 28, pages 54-55, January 1931. The apparatus was originally designed for testing liquid oils but by addition of suitable feeding appliances which feed grease on the test pieces, the apparatus has been rendered useful for testing greases. A description of its use for testing greases is given in the Journal of the Institution of Petroleum, volume 26, Number 200, pages 273-283, June 1940.

The greases prepared by Processes A and B described hereinabove are compared in the table.

Table

| Grease                                                 | Process A | Process B |
|--------------------------------------------------------|-----------|-----------|
| <b>Storage Stability—</b>                              |           |           |
| Original Penetration, ASTM 77° F.:                     |           |           |
| Unworked.....                                          | 345       | 363       |
| Worked.....                                            | 325       | 343       |
| Penetration After Storage for 3 Months<br>ASTM 77° F.: |           |           |
| Unworked.....                                          | 344       | 385       |
| Worked.....                                            | 318       | 355       |
| Timken O. K. Load—Pounds.....                          | 50        | 40        |
| <b>Shear Stability Tests—</b>                          |           |           |
| For 3½ hours at 2,000 pounds per square inch gauge:    |           |           |
| Worked Penetration ASTM 77° F. ....                    | 352       | 400       |

It will be noted from the table that the grease prepared by the method of this invention is superior to the one prepared using prior art processes procedure with respect to storage stability, shear stability and load rating without bearing failure. Moreover, the method of this invention permits a reduction in manufacturing time using the same grease kettles from 22 hours by prior art procedure to 10-12 hours by the procedure of this invention, thereby doubling the capacity of the grease manufacturing plant. The method of this invention eliminates the necessity of preparing the lead soap separately and thereby eliminates the separate apparatus heretofore required for that step. The method of this invention also permits the introduction of the total lime requirement in the initial kettle charge thereby eliminating the necessity for subsequent lime addition to the partially manufactured grease.

The process above described is also useful in preparing greases based upon the soaps or other alkaline earth metals, such as barium, magnesium and strontium.

In this case a barium base grease containing lead soaps and barium acetate was prepared. The formulation was as follows:

### EXAMPLE III

| Ingredient:                                                  | Percent by weight |
|--------------------------------------------------------------|-------------------|
| Acidless tallow.....                                         | 7.0               |
| Oleic acid.....                                              | 3.6               |
| Barium hydroxide (dry powder, 95% Ba(OH) <sub>2</sub> )..... | 6.6               |
| Glycerine.....                                               | 1.0               |
| Acetic acid.....                                             | 1.8               |
| Litharge (slurry in oil).....                                | 1.8               |
| Sulfurized fatty oil (10% S).....                            | 4.0               |
| Mineral oil (100° S. U. V. @ 100° F.).....                   | 37.1              |
| Mineral oil (block oil, 200° S. U. V. @ 100° F.).....        | 37.1              |

The above ingredients were compounded together using the same procedure as outlined in Example I, above. The resulting grease was of good consistency, stable in service under high unit pressures, and capable of use at reasonably high temperatures.

Its properties were:

Timken O. K. load, pounds..... 40  
A. S. T. M. drop point..... °F. 237

Storage stability:

Original penetration, A. S. T. M.,  
77° F.—

    Unworked ..... 315  
    Worked ..... 340

Penetration after storage, A. S. T. M.,  
77° F.—

    After 12 days:  
        Unworked ..... 280  
        Worked ..... 353

    After 16 days:  
        Unworked ..... 280  
        Worked ..... 345

Shear stability test:  
3½ hours at 2000 pounds per square inch gauge

Worked penetration, A. S. T. M.,  
77° F. .... 370

Similarly, competent greases may be prepared utilizing the soaps of magnesium and strontium.

It will, of course, be realized that various modifications which will readily appear to those skilled in the art may be made in the procedure outlined hereinabove without departure from the spirit and scope of this invention. Moreover, certain of the constituents mentioned may be eliminated or replaced by substitutes and the various proportions may be changed within limits depending upon the desired characteristics of the final grease. In general, the following ranges, limits and variations in the procedure are intended to be within the scope of this invention.

(1) The tallow and/or candelilla wax may be replaced by other suitable saponifiable materials such as lard oil, hog fat, high molecular weight organic cuts such as stearic and oleic acids, rosin and related products, beeswax, sperm oil, degras, etc. The molecular weight of these saponifiable materials should in general be greater than about 200. The saponifiable materials added should be less than about 30 percent by weight of the total material going into the grease composition.

(2) The non-corrosive sulfurized fatty oil may be prepared by methods other than that outlined in Example I. Suitable sulfurized fatty oils may be prepared by heating sulfur in varying proportions ranging up to about ten to fifteen percent by weight of the oil with sperm oil, corn oil, lard oil, cottonseed oil and the like by procedure well known to the art. The amount of sulfurized oil added to the grease composition may be controlled, in case a grease not containing sulphur in corrosive amounts is desired, to provide a grease in which the sulfur compound content measured as sulfur amounts to about 0.25 to 4.0 percent by weight of the grease. The presence of these sulfur compounds in the grease is important in that they improve its load bearing characteristics.

(3) The amount of lead added in producing the grease measured as PbO should be broadly within the range 0.5 to 5.0 percent of the total materials added and preferably within the range 1 to 2.0 percent by weight thereof. In the case